

No. 671,882.

Patented Apr. 9, 1901.

O. FULTON & M. GILLARD.

PHOTOGRAPHIC PRINTING SURFACE AND METHOD OF MAKING SAME.

(No Model.)

(Application filed July 23, 1900.)

Fig. 1.



Fig. 2.



Witnesses.

Robert Everett,

W. K. Keeler

Inventors.

Otto Fulton

Mountsler Gillard.

By James L. Norris.

Atty.

# UNITED STATES PATENT OFFICE.

OTTO FULTON AND MOUNTSTEVEN GILLARD, OF PORT ELIZABETH, CAPE COLONY.

## PHOTOGRAPHIC-PRINTING SURFACE AND METHOD OF MAKING SAME.

SPECIFICATION forming part of Letters Patent No. 671,882, dated April 9, 1901.

Application filed July 28, 1900. Serial No. 24,591. (No specimens.)

*To all whom it may concern:*

Be it known that we, OTTO FULTON and MOUNTSTEVEN GILLARD, photographers, subjects of the Queen of Great Britain, residing 5 at Main street, Port Elizabeth, Cape Colony, have invented certain new and useful Improvements in Photographic-Printing Surfaces and Methods of Producing the Same, of which the following is a specification.

10 This invention relates to the production of photographic-printing surfaces in a simple, economical, and expeditious manner without requiring any special ability on the part of the person making and using the same. Furthermore, the printing-surfaces are so formed 15 that a great number of prints or impressions can be obtained therefrom without the aid of any expensive apparatus or machinery upon any desired material and in various colors or 20 tints. Moreover, the said printing-surfaces do not materially deteriorate by remaining out of use for a considerable length of time.

According to our invention we obtain what is known as a "collotype" printing-surface 25 upon a sheet of celluloid or similar non-flaccid but semirigid waterproof material which is elastic and flexible, so that it can be freely handled like a card and printed from without either being cemented to a mounting-block 30 or stretched at the two ends, as is usually necessary with films that are flaccid. One of the surfaces of the aforesaid sheet must be rough or matte, and to this surface we apply a gelatinous solution, and we dry the coated sheet 35 in such a manner that perfect adhesion of the dried gelatinous film or coating to the said sheet will be insured, as hereinafter explained. It is important that the gelatinous solution from which the said film is formed should 40 contain formalin, citric acid, (together or separately,) or some other substance that will tend to harden the film. The said celluloid sheet provided with its gelatinous film is then ready to be sensitized by means of a solution of a bi- 45 chromate or a chromate in the way well known to collotype printers, after which it is placed in an ordinary printing-frame, together with a negative, and exposed to light in the manner which is well understood. After exposing the 50 same for a sufficient length of time the negative is removed from the frame and the back

of the sheet is exposed to the light for a short time in order to completely indurate that portion of the gelatinous film which is in immediate contact with the said sheet. After this 55 operation the sheet is soaked in water and dried. The surface upon which the photographic picture has been obtained is then treated with a mixture of glycerin, ammonia, and water. After this treatment and when 60 all superfluous moisture has been removed the sheet is ready to receive the printing-ink, which may be applied in any ordinary and well-known manner.

In the drawings accompanying this specification, Figure 1 is an elevation, broken away, of our improved photographic-printing surface; and Fig. 2 is a plan of a mask used in connection therewith.

Referring to the drawings by reference-numbers, 1 indicates a rough or matte sheet of celluloid; 2, the gelatinous film; 3, the sensitized film, and 4 the preservative coating.

The reference-numeral 5 indicates a mask used in the preparation of the printing-surface. This mask may be of any desired form.

The components of the gelatinous film, the sensitized coating, and the preservative will be hereinafter explicitly set forth.

In carrying our invention into practice we 80 take a sheet of celluloid which is rough or matte on one side and thick enough to be rigid in the sense in which a sheet of ordinary thin card is rigid. The thickness of the sheet we prefer to use is about one-hundredth of an 85 inch. Extremely thin celluloid like that used in photographic-roll holders is not satisfactory, neither are sheets the thickness of which reaches one-thirteenth of an inch. It is necessary that the natural translucency of the 90 sheet of celluloid employed shall not be entirely destroyed by the addition or incorporation of pigments. In order to coat the celluloid sheet evenly with the gelatinous film, we proceed as follows, viz: A perfectly flat 95 support preferably consisting of plate-glass is coated with an adhesive solution composed of water, eight (8) ounces; glue, (French,) one-half ( $\frac{1}{2}$ ) ounce; glycerin, three (3) ounces; formalin, sixty (60) minims. Such solution 100 is prepared in the following manner: The glue in small pieces is placed in a vessel con-

taining the water and allowed to remain there-  
in for some hours, and when the glue is thor-  
oughly softened the vessel is gently warmed  
until the glue is dissolved. The formalin and  
5 glycerin mixed together are then added  
slowly, the whole being well stirred. The so-  
lution is then filtered through a piece of mus-  
lin. During the filtering it is desirable to  
10 warm the muslin and the vessel intended to  
contain the adhesive solution. A quantity  
of this adhesive solution is then poured upon  
the plate-glass and evenly spread over the  
entire surface by the aid of a warmed glass  
15 rod to form a thin coating. The support thus  
coated is then placed upon a perfectly-level  
slab and allowed to remain for a few minutes  
until the adhesive surface has set and cooled.  
The celluloid sheet is next applied to the ad-  
hesive surface of the support and with the  
20 rough side upward is slightly pressed down  
onto the adhesive surface by the hand with  
the aid of a cloth, great care being taken that  
no air-bubbles are left between the celluloid  
sheet and the adhesive surface. When the  
25 celluloid sheet has been thus mounted upon  
the adhesive surface, we coat the said sheet  
with a gelatinous mixture which is prepared  
as follows: Gelatin, one hundred and eighty  
(180) grains; formalin, fifteen (15) minimis; cit-  
30 ric acid, five (5) grains; water, five (5) ounces.  
The gelatin is cut into small pieces, placed in  
four ounces of the water, and allowed to soak.  
It is then warmed to a temperature of about  
120° Fahrenheit and stirred until dissolved.  
35 The vessel containing the mixture should be  
heated in a water-bath and not directly by  
a flame. When the gelatin has been com-  
pletely melted, the formalin and citric acid are  
mixed with the remaining ounce of water and  
40 this liquid is added slowly to the gelatinous  
mixture and at the same time is well stirred.  
The solution is afterward filtered with simi-  
lar precautions to those already mentioned.  
We now coat the sheet of celluloid while it is  
45 still mounted on the aforesaid support by  
pouring upon it a sufficient quantity of the  
solution to cover the sheet with a thin layer,  
the solution being spread thereon by the aid  
of a warmed glass rod. A surface eight and  
50 one-half inches by eight and one-half inches  
will ordinarily require about one ounce of the  
gelatinous solution. The solution is now al-  
lowed to set while the celluloid is still on the  
level adhesive support, and the coating is af-  
55 terward dried at a temperature of about 85°  
Fahrenheit. Provided that the coating has  
thoroughly set, there is no objection to placing  
the support vertically when drying. When  
perfectly dry, the coated celluloid sheet, with  
60 its gelatinous film, is removed from the ad-  
hesive support by drawing it off by one of its  
corners. It will be found advantageous to  
place a fresh sheet of celluloid upon the ad-  
hesive support immediately after the removal  
65 of the first-mentioned one, so as to protect  
the adhesive surface from air and dust. It  
can then be used a great number of times or

after remaining disused for a considerable  
length of time. The coated celluloid sheet  
thus obtained is then placed in a sensitizing  
70 solution or bath, with the gelatinous film up-  
permost, this solution being an ordinary bi-  
chromate or chromate sensitizing-bath—such  
as potassium bichromate, one (1) ounce; am-  
monium hydrate, ten (10) drops; water, forty  
75 (40) ounces. In hot weather it may be nec-  
essary to cool the sensitizing solution. The  
sheet is allowed to remain in the sensitizing  
solution for about two and one-half minutes.  
It is then removed and placed between folds  
80 of damp blotting-paper for the purpose of re-  
moving superfluous moisture, and the sheet  
is then dried in the dark. When perfectly  
dry, the sheet is placed, with the photo-  
graphic negative, in an ordinary printing-  
85 frame, with the yellow or sensitized side of  
the celluloid sheet against the negative. Be-  
fore printing, however, we prefer to place be-  
tween the glazed opening of the printing-  
frame and the negative a mask, so as to leave  
90 a margin around the celluloid sheet of about  
half an inch, this mask being similar to the  
“safe edge” used by carbon-printers. The  
margin may be broader, but should not be  
narrower. We then expose the negative and  
95 the celluloid sheet in a soft light or in the  
shade until the said celluloid sheet exhibits  
the picture in all details and graduations.  
We then remove the negative, still keeping  
the mask in the frame. We then reverse the  
100 celluloid sheet, so that its unsensitized side  
is toward the glass of the frame. The sheet  
is then exposed to the light for about three  
minutes (or generally about one-fifth of the  
time of the chief exposure) to harden the  
105 gelatinous material which is in immediate  
contact with the celluloid sheet. We now  
remove the celluloid sheet from the print-  
ing-frame and place it with the yellow side  
uppermost in a bath of water, changing the  
110 water about every five or ten minutes till  
all the free bichromate is washed out and no  
trace of yellow left. The sheet is then re-  
moved from the water, and after the super-  
fluous moisture has been removed by a cloth  
115 the sheet is allowed to dry. Upon the dried  
sheet we pour a solution consisting of gly-  
cerin, ten (10) ounces; ammonium hydrate,  
one quarter ( $\frac{1}{4}$ ) ounce; water, five (5) ounces.  
The quantity of this solution used is suffi-  
120 cient to just cover the picture and a small  
margin around the same. It is allowed to  
stand for forty or fifty minutes, according to  
the softness or hardness of the negative em-  
ployed. After sponging it and removing all  
125 superfluous moisture the sheet is then ready  
to receive the printing-ink, which may be the  
ordinary lithographic or typographic kind  
mixed with varnish. The ink may be applied  
to the printing-surface of the celluloid sheet  
130 in any ordinary manner. The impressions  
from the printing-surface can be made on any  
kind of material and in almost any color and  
with only a slight pressure obtained by a

hand-roller or a letter-press or in any other convenient manner.

From time to time the printing-block should be sponged with a mixture of glycerin and water in about equal proportions.

What we claim, and desire to secure by Letters Patent of the United States, is—

1. The herein-described method of obtaining a photographic-printing surface, consisting in first coating a sheet of suitable material with a hardened gelatinous film having a safe edge, sensitizing the said coating and exposing and then reversing the sheet to allow the light to harden the whole film excepting the safe edge.

2. The herein-described method of obtaining a photographic-printing surface, consisting in coating a sheet of suitable material with a gelatinous film, sensitizing the said film, masking a portion of said film while printing to form a safe edge and finally hardening the gelatinous film.

3. A photographic-printing surface, consisting of a sheet of celluloid having a hardened gelatinous film with a safe edge.

4. The herein-described method of obtaining a photographic-printing surface, consisting of placing a sheet of suitable material

upon a support having an adhesive surface, coating the outer face of said sheet with a 30 gelatinous film, sensitizing the said film, masking a portion of said film while printing from a negative to form a safe edge, and finally hardening said gelatinous film.

5. The herein-described method of obtaining a photographic-printing surface, consisting of placing a sheet of celluloid upon an adhesive surface, coating the outer face of said sheet with a solution consisting of gelatin, formalin, citric acid and water to form a 40 gelatinous film, sensitizing the said film, masking a portion of said film while printing to form a safe edge, and finally hardening said gelatinous film.

6. A photographic-printing surface, consisting of a sheet of celluloid having a hardened sensitized film of gelatin, formalin and citric acid with a safe edge.

In testimony whereof we have hereunto set our hands, in presence of two subscribing 50 witnesses, this 18th day of December, 1899.

OTTO FULTON.

MOUNTSTEVEN GILLARD.

Witnesses:

J. COLLINS,  
FRED C. HARRIS.